# EUROPEAN PATENT SPECIFICATION

(11) **EP 2 860 291 B1**
(45) Date of publication and mention of the grant of the patent: **08.01.2020**
(21) Application number: 13803425.1
(22) Date of filing: 30.05.2013
(51) Int. Cl.: C25C 3/12, B22D 25/00, C22C 9/00, C22C 9/06, C22C 19/03, C22C 30/02, C22C 30/04, C22C 38/00, C22C 38/06, C22C 38/08, C22C 38/16

(54) **INERT ALLOY ANODE USED FOR ALUMINUM ELECTROLYSIS AND PREPARATION METHOD THEREFOR**
INERTE ANODE FÜR ALUMINIUMELEKTROLYSE UND HERSTELLUNGSVERFAHREN DAFÜR
ANODE EN ALLIAGE INERTE UTILISÉE POUR L'ÉLECTROLYSE D'ALUMINIUM ET PROCÉDÉ DE PRÉPARATION ASSOCIÉ

(30) Priority: 11.06.2012 CN 201210188424; 23.01.2013 CN 201310024019
(43) Date of publication of application: 15.04.2015
(73) Proprietor: Inner Mongolia United Industrial Co. Ltd., Inner Mongolia 010020 (CN)
(72) Inventor: SUN, Songtao, Hohhot Inner Mongolia 010020 (CN); FANG, Yulin, Hohhot Inner Mongolia 010020 (CN)
(74) Representative: Groth & Co. KB
(86) International application number: PCT/CN2013/076441
(87) International publication number: WO 2013/185539

(56) References cited:
- WO-A1-98/12363
- CN-A- 101 717 969
- CN-A- 101 824 631
- CN-A- 102 011 144
- US-A- 5 904 828
- US-A1- 2005 000 823
- US-A1- 2005 205 431
- US-A1- 2005 205 431
- US-A1- 2007 278 107
- US-A1- 2007 278 107
- US-B1- 6 361 680
- LI, JIE ET AL.: 'Development of anode material for electrolytic aluminum' CHEMICAL ENGINEER no. 12, December 2008, pages 26 - 29, XP008175666

## Description

### Field of the Invention

The present invention relates to an inert alloy anode for aluminum electrolysis and a preparing method thereof, belonging to the field of aluminum electrolysis industry.

### Background of the Invention

Aluminum electrolysis refers to acquisition of aluminum by alumina electrolysis. In the prior art, a traditional Hall-Heroult molten salt aluminum electrolysis process is typically adopted for aluminum electrolysis, this process is featured by use of a cryolite-alumina molten salt electrolysis method in which cryolite Na₃AlF₆ fluoride salt melt is taken as flux, Al₂O₃ is dissolved in the fluoride salt, a carbon body is taken as an anode, aluminum liquid is taken as a cathode, and electrolytic aluminum is obtained by performing electrochemical reaction at the anode and cathode of the electrolytic cell at a high temperature ranging from 940°C to 960°C after a strong direct current is introduced. In the traditional aluminum electrolysis process, a carbon anode is ceaselessly consumed in the electrolysis process, thus constant replacement for the carbon anode is required; moreover, carbon dioxide, carbon monoxide, toxic fluorine hydride and other waste gases are continuously generated at the anode during alumina electrolysis, emission of these gases into environment will be harmful to environment and health of human and livestock, so that the waste gases generated by aluminum electrolysis need to be purified before emission, which accordingly increases the investment cost of the alumina electrolysis production process.

Consumption of the anode material in the process of aluminum electrolysis is mainly caused by oxidization reaction, in the electrolysis process, of the carbon anode material used in the traditional Hall-Heroult process. Therefore, many domestic and foreign researchers have commenced the study on anode material in order to reduce consumption of the anode material in the process of aluminum electrolysis and simultaneously lessen waste gas emission.

WO 98/12363A1 discloses a metal alloy consisting of: 5-20, preferably 5-20 wt% of Fe; 0-15, preferably 5-15 wt% of Cu; 50-90, preferably 60-80 wt% of Ni; 3-20, preferably 3-10 wt% of Al; 0.5-5, preferably 0.5-5 wt % of at least one additive element from the group consisting of Si, Sn, Zn, V, In, Hf, W, elements from lanthanide series starting from Pr and misch metal and optionally other additives.

CN 102011144A relates to nickel-based alloy material suitable for inert anode of metal molten salt electrolyzer, comprising: 15-50 wt% of Fe, 5-20 wt% of Cu, 0-10 wt% of Sn, 3-15 wt% of Al, 0.1-1 wt% of Si, 0.05-5 wt% of rare earth elements selected from Sc, Y, La, Ce or Yb and the balance of Ni. The Example 4 of CN 102011144A discloses an alloy anode involving Fe, Cu, Ni and Sn, in detail, comprising the following components by weight: 45% of Fe, 8% of Al, 8% of Cu, 5.0% of Y, 0.6% of Sn, 0.1% of Si, and Ni for making up to 100%. In the electrolysis experiments of CN 102011144A, the electrolysis voltage is in the range of 3.6-4.0V.

US 2007/0278107A1 discloses an inert alloy anode, comprising 10-70wt% of Cu, 15-50wt% of Ni, 1-15 wt% of Sn, and the balance being iron; and preferably comprising 10-20wt% of Cu, 20-30 wt% of Ni, 2-5wt% of Sn, 50-70wt% of Fe. The anode according to US 2007/0278107 has an average cell voltage of 4.17V or 4.08V during the electrolysis process.

US 2005/0205431A1 discloses a metal alloy consisting of: 20-60, preferably 35-60 wt% of Ni; 5-15, preferably 6-12 wt% of Cu; 1.5-5, preferably 1.5-4 wt% of Al; 0-2, preferably 0.2-0.5 wt% of one or more rare earth metals, in particular yttrium; 0-2, preferably 0.5-1.5 wt% of further elements, in particular manganese, silicon and carbon; and the balance being iron.

The Chinese patent document CN102230189A discloses a metal ceramic inert anode material for aluminum electrolysis, which is obtained by the steps of preparing an NiO-NiFe₂O₄ metal ceramic matrix from raw materials including Ni₂O₃ and Fe₂O₃ and then adding metal copper powder and nano NiO, and which has an electric conductivity as high as 102Ω⁻¹•cm⁻¹. In the above art, the anode material with metal ceramic as the matrix, though hardly reacting with electrolyte, is large in resistance and high in overvoltage, which results in large power consumption of the process and high cost in the process of aluminum electrolysis; furthermore, the anode material with metal ceramic as the matrix has poor thermal shock resistance and consequently is liable to brittlement during use; and in addition, the processability in use of the anode made from the above materials is poor just because the anode material having the metal ceramic matrix is liable to brittlement, as a result, the anode in any shape cannot be obtained.

To solve the problem that the anode material having the metal ceramic matrix is low in electric conductivity and brittle in structure, some researchers have brought forward use of alloy metals as the anode material, in order to improve the electric conductivity of the anode material and simultaneously improve the processability of the anode material. Disclosed in Chinese patent document CN1443877A is an inert anode material applied to aluminum, magnesium, rare earth and other electrolysis industries, this material is formed by binary or multi-element alloy composed of chromium, nickel, ferrum, cobalt, titanium, copper, aluminum, magnesium and other metals, and the preparation method thereof is a method of smelting or powder metallurgy. The prepared anode material is good in electric and thermal conductivity and generates oxygen in the electrolysis process, wherein in Example 1, an anode is made of the alloy material composed of 37wt% of cobalt, 18wt% of copper, 19wt% of nickel, 23wt% of ferrum and 3wt% of silver and is used for aluminum electrolysis, the anode has a current density of 1.0A/cm² in the electrolysis process at 850°C and the cell voltage is steadily maintained within a range from 4.1V to 4.5V in the electrolysis process, the prepared aluminum has a purity of 98.35%.

In the case that the alloy composed of a plurality of metals, including chromium, nickel, ferrum, cobalt, titanium, copper, aluminum and magnesium, is used as the anode material for aluminum electrolysis in the above art, this alloy anode material has higher electric conductivity than the anode ceramic matrix anode material, can be processed in any shape by a smelting or powder metallurgy method and is hardly consumed in the electrolysis process compared with the carbon anode material. However, a large amount of expensive metal materials are used in preparation of the alloy anode in the above art to result in high cost of the anode material, and thus this alloy anode fails to meet the demand on industrial cost; moreover, the alloy anode prepared from the above metal components is low in electric conductivity and high in overvoltage, so that the power consumption of the process is increased, thus the alloy anode cannot meet the needs of the aluminum electrolysis process.

In addition, an oxide film is generated on the surface of the prepared alloy anode in the prior art, and if this oxide film is destroyed, the anode material exposed to the surface will be oxidized as a new oxide film. The oxide film on the surface of the alloy anode in the above art has low oxidization resistance and is further liable to oxidization reaction to generate products that are likely to be corroded by electrolyte, and the oxide film with low stability is liable to fall off the anode electrode in the electrolysis process; after the previous oxide film is corroded or falls off, the material of the alloy anode exposed to the surface will create a new oxide film by reaction with oxygen, such replacement between new and old oxide films results in continuous consumption and poor corrosion resistance of the anode material as well as short service life of electrodes; furthermore, the corroded or falling oxide film enters into liquid aluminum in the electrolysis process of alumina to degrade the purity of the final product aluminum, as a result, the manufactured aluminum product cannot meet the demand of national standards and accordingly cannot be directly used as a finished product.

### Summary of the Invention

The first technical problem to be solved by the present invention is that the alloy anode in the prior art is expensive in metal materials used, high in process cost, low in electric conductivity and high in overvoltage, as a result, power consumption of the process is increased; therefore, provided is an inert alloy anode for aluminum electrolysis with low cost and overvoltage, and preparing methods thereof, according to the appended claims.

Simultaneously, the second technical problem to be solved by the present invention is that, an oxide film on the surface of the alloy anode in the prior art is low in oxidation resistance and liable to fall off, which leads to continuous consumption of the alloy anode and poor corrosion resistance, furthermore, the corroded or falling oxide film enters into liquid aluminum to degrade the purity of the final product aluminum; therefore, provided is an inert alloy anode for aluminum electrolysis, which is strong in oxidization resistance of the oxide film formed on the surface and not liable to fall off so as to improve the corrosion resistance thereof and the purity of the product aluminum, and a preparing method of the inert alloy anode.

To solve the aforementioned technical problems, the present invention provides an inert alloy anode for aluminum electrolysis, which contains Fe and Cu as primary components, and further contains Sn.

The mass ratio of Fe to Cu to Sn is (23-40): (36-60): (0.2-5) or (40.01-80): (0.01-35.9): (0.01-0.19).

The inert alloy anode further contains Ni.

The mass ratio of Fe to Cu to Ni to Sn is (23-40): (36-60): (14-28): (0.2-5) or (40.01-80): (0.01-35.9): (28.1-70): (0.01-0.19).

The inert alloy anode is composed of Fe, Cu, Ni and Sn, wherein the content of Fe is 23-40wt%, the content of Cu is 36-60wt%, the content of Ni is 14-28wt% and the content of Sn is 0.2-5wt%, or the content of Fe is 40.01-71.88wt%, the content of Cu is 0.01-31.88wt%, the content of Ni is 28.1-59.97wt% and the content of Sn is 0.01-0.19wt%.

The inert alloy anode further contains Al.

The inert alloy anode is composed of Fe, Cu, Ni, Sn and Al, wherein the content of Fe is 23-40wt%, the content of Cu is 36-60wt%, the content of Ni is 14-28wt%, the content of Al is more than zero and less than or equal to 4wt% and the content of Sn is 0.2-5wt%, or the content of Fe is 40.01-71.88wt%, the content of Cu is 0.01-31.88wt%, the content of Ni is 28.1-59.97wt%, the content of Al is more than zero and less than or equal to 4wt% and the content of Sn is 0.01-0.19wt%.

The inert alloy anode further contains Y.

The inert alloy anode is composed of Fe, Cu, Ni, Sn, Al and Y, wherein the content of Fe is 23-40wt%, the content of Cu is 36-60wt%, the content of Ni is 14-28wt%, the content of Al is more than zero and less than or equal to 4wt%, the content of Y is more than zero and less than or equal to 2wt% and the content of Sn is 0.2-5wt%, or the content of Fe is 40.01-71.88wt%, the content of Cu is 0.01-31.88wt%, the content of Ni is 28.1-59.97wt%, the content of Al is more than zero and less than or equal to 4wt%, the content of Y is more than zero and less than or equal to 2wt% and the content of Sn is 0.01-0.19wt%.

A preparing method of the inert alloy anode comprises the following steps:
melting and uniformly mixing the metals Fe, Cu and Sn, and then rapidly casting and cooling the mixture to obtain the inert alloy anode;
or, melting the metals Fe, Cu and Sn at first, then adding and melting the metal Al or Y, and uniformly mixing, or adding and melting the metal Al at first, then adding and melting the metal Y, uniformly mixing, and rapidly casting and cooling the mixture to obtain the inert alloy anode;
or, melting and mixing the metals Fe, Cu, Ni and Sn and then casting the mixture to obtain the inert alloy anode;
or, melting the metals Fe, Cu, Ni and Sn at first, then adding and melting the metal Al or Y, and uniformly mixing, or adding and melting the metal Al at first, then adding and melting the metal Y, uniformly mixing, and casting the mixture to obtain the inert alloy anode.

Compared with the prior art, the inert alloy anode for aluminum electrolysis in the present invention has the beneficial effects below:
(1) The inert alloy anode for aluminum electrolysis in the present invention contains Fe and Cu as primary components, and further contains Sn. The inert alloy anode with the above components is low in cost, low in overvoltage and small in power consumption of the aluminum electrolysis process; the anode material is alloy composed of Fe, Cu and Sn, so an oxide film formed on the surface of the inert alloy anode in the electrolysis process is high in oxidation resistance and is hardly corroded by electrolyte, and the formed oxide film is stable and not liable to fall off, therefore, the inert alloy anode is imparted with quite high oxidation resistance and corrosion resistance. It is precisely because of high oxidation resistance and corrosion resistance of the inert alloy anode, impurities entering into liquid aluminum, which are generated by corrosion or falling off of the anode material, are avoided, so as to ensure the purity of aluminum products, that is, the purity of the produced aluminum can reach 99.8%. The following problems are avoided: the alloy anode in the prior art has high cost and overvoltage and large power consumption of process, the oxide film on the alloy surface is low in oxidation resistance and liable to fall off, which leads to continuous consumption of the alloy anode and poor corrosion resistance, furthermore, the corroded or falling oxide film enters into liquid aluminum to degrade the purity of the final product aluminum.
(2) The inert alloy anode for aluminum electrolysis in the present invention is composed of Fe, Cu, Ni and Sn, wherein the content of Fe is 23-40wt%, the content of Cu is 36-60wt%, the content of Ni is 14-28wt% and the content of Sn is 0.2-5wt%, or the content of Fe is 40.01-71.88wt%, the content of Cu is 0.01-31.88wt%, the content of Ni is 28.1-59.97wt% and the content of Sn is 0.01-0.19wt%.
   The alloy anode in the present invention contains Fe and Cu as primary components, their content proportions are high, so the material cost of the inert alloy anode is reduced, meanwhile, the inert alloy anode composed of the aforementioned metal components is high in electric conductivity and has a cell voltage as low as 3.1V to 3.4V, power consumption for aluminum electrolysis is small, the power consumption for per ton of aluminum is not more than 11000kw•h, so the production cost of electrolytic aluminum is low. The following problems are avoided: a large quantity of expensive metal materials are used in the anode material in the prior art, resulting in increase of the anode production cost; the prepared alloy anode is low in electric conductivity, large in power consumption for aluminum electrolysis and increased in cost, and cannot be applied to industrial production. The added metal Ni is capable of promoting firmer combination among other types of metals, and the added metal Sn ensures that an oxide film with high oxidization resistance, good corrosion resistance and high stability can be formed on the surface of the inert alloy anode in the electrolysis process.
(3) The inert alloy anode for aluminum electrolysis in the present invention is composed of Fe, Cu, Ni, Sn, Al and Y, wherein the content of Fe is 23-40wt%, the content of Cu is 36-60wt%, the content of Ni is 14-28wt%, the content of Al is more than zero and less than or equal to 4wt%, the content of Y is more than zero and less than or equal to 2wt% and the content of Sn is 0.2-5wt%, or the content of Fe is 40.01-71.88wt%, the content of Cu is 0.01-31.88wt%, the content of Ni is 28.1-59.97wt%, the content of Al is more than zero and less than or equal to 4wt%, the content of Y is more than zero and less than or equal to 2wt% and the content of Sn is 0.01-0.19wt%. Similarly, the aforementioned inert alloy anode has the advantages of low material cost and high electric conductivity, in addition, the metal Al contained in the aforementioned inert alloy anode plays a role of oxidization resistance and can serve as a reducing agent for metallothermic reduction reaction with a metal oxide in the inert anode alloy, thus ensure the percentage of the primary components in the inert alloy anode, meanwhile, the added metal Y can be used for controlling a crystal structure for anode material formation in the preparation process of the inert anode, achieving the anti-oxidization purpose.
(4) The inert alloy anode for aluminum electrolysis in the present invention has a melting point of 1360-1386°C, a specific resistivity of 68-76.8µΩ•cm at 20°C and a density of 8.1-8.3g/cm³. The prepared inert alloy anode has a quite high melting point and accordingly can meet the demand of aluminum electrolysis on high temperature environment; furthermore, the aforementioned inert alloy anode has a quite low overvoltage, so power consumption of the aluminum electrolysis process can be reduced; the prepared inert alloy anode is even in texture and has a density within a range from 8.1 g/cm³ to 8.3g/cm³, in this way, stable service property of the inert alloy anode is guaranteed.
(5) The preparing method of the inert alloy anode comprises the following steps: melting and uniformly mixing the metals Fe, Cu and Sn, and then rapidly casting and cooling the mixture to obtain the inert alloy anode; or, melting the metals Fe, Cu and Sn at first, then adding and melting the metal Al or Y, and uniformly mixing, or adding and melting the metal Al at first, then adding and melting the metal Y, uniformly mixing, and rapidly casting and cooling the mixture to obtain the inert alloy anode; or, melting and mixing the metals Fe, Cu, Ni and Sn and then casting the mixture to obtain the inert alloy anode; or, melting the metals Fe, Cu, Ni and Sn at first, then adding and melting the metal Al or Y, and uniformly mixing, or adding and melting the metal Al at first, then adding and melting the metal Y, uniformly mixing, and casting the mixture to obtain the inert alloy anode. The aforementioned inert alloy anode is simple in preparation process and can be prepared in any shape according to the actual needs. During preparation of the alloy containing the metals Al and Y, Al is added at first to prevent other molten metal components from being oxidized, and then, Y is added and molten to finally obtain the alloy having a desired crystal form.

For more easily understanding the technical solution of the present invention, further description will be made below to the technical solution of the present invention in conjunction with the embodiments.

### Detailed Description of the Embodiments

### Embodiment 1

23 parts by weight of Fe metal blocks, 60 parts by weight of Cu metal blocks and 0.2 parts by weight of Sn metal blocks are molten and then uniformly mixed under high-speed electromagnetic stirring, the mixture is rapidly cast and then rapidly cooled at a speed of 20-100°C/s to obtain an inert alloy anode 1 which is homogeneous in texture. The inert alloy anode has a density of 8.3g/cm³, a specific resistivity of 62µΩ•cm and a melting point of 1400°C.

### Embodiment 2

40 parts by weight of Fe metal blocks, 36 parts by weight of Cu metal blocks and 5 parts by weight of Sn metal blocks are molten and then uniformly mixed under high-speed electromagnetic stirring, the mixture is rapidly cast and then rapidly cooled at a speed of 20-100°C/s to obtain an inert alloy anode 2 which is homogeneous in texture. The inert alloy anode has a density of 7.8g/cm³, a specific resistivity of 82µΩ•cm and a melting point of 1369°C.

### Embodiment 3

30 parts by weight of Fe metal blocks, 45 parts by weight of Cu metal blocks and 3 parts by weight of Sn metal blocks are molten and then uniformly mixed under high-speed electromagnetic stirring, the mixture is rapidly cast and then rapidly cooled at a speed of 20-100°C/s to obtain an inert alloy anode 3 which is homogeneous in texture. The inert alloy anode has a density of 7.9g/cm³, a specific resistivity of 86µΩ•cm and a melting point of 1390°C.

### Embodiment 4

30 parts by weight of Fe metal blocks, 50 parts by weight of Cu metal blocks, 20 parts by weight of Mo and 5 parts by weight of Sn metal blocks are molten and then cast to obtain an inert alloy anode 4. The inert alloy anode has a density of 8.2g/cm³, a specific resistivity of 78µΩ•cm and a melting point of 1370°C.

### Embodiment 5

23 parts by weight of Fe metal blocks, 60 parts by weight of Cu metal blocks, 14 parts by weight of Ni and 3 parts by weight of Sn metal blocks are molten and then cast to obtain an inert alloy anode 5. The inert alloy anode has a density of 8.3g/cm³, a specific resistivity of 68µΩ•cm and a melting point of 1360°C.

### Embodiment 6

40 parts by weight of Fe metal blocks, 36 parts by weight of Cu metal blocks, 19 parts by weight of Ni and 5 parts by weight of Sn metal blocks are molten and then cast to obtain an inert alloy anode 6. The inert alloy anode has a density of 8.1g/cm³, a specific resistivity of 76.8µΩ•cm and a melting point of 1386°C.

### Embodiment 7

25 parts by weight of Fe metal blocks, 46.8 parts by weight of Cu metal blocks, 28 parts by weight of Ni and 0.2 parts by weight of Sn metal blocks are molten and then cast to obtain an inert alloy anode 7. The inert alloy anode has a density of 8.2g/cm³, a specific resistivity of 72µΩ•cm and a melting point of 1350°C.

### Embodiment 8

23 parts by weight of Fe metal blocks, 60 parts by weight of Cu metal blocks, 14 parts by weight of Ni and 3 parts by weight of Sn metal blocks are molten and then cast to obtain an inert alloy anode 8. The inert alloy anode has a density of 8.1g/cm³, a specific resistivity of 70µΩ•cm and a melting point of 1330°C.

### Embodiment 9

40 parts by weight of Fe metal blocks, 36 parts by weight of Cu metal blocks, 19 parts by weight of Ni and 5 parts by weight of Sn metal blocks are molten and then cast to obtain an inert alloy anode 9. The inert alloy anode has a density of 8.2g/cm³, a specific resistivity of 73µΩ•cm and a melting point of 1340°C.

### Embodiment 10

24 parts by weight of Fe metal blocks, 47.8 parts by weight of Cu metal blocks, 28 parts by weight of Ni and 0.2 parts by weight of Sn metal blocks are molten and then cast to obtain an inert alloy anode 10. The inert alloy anode has a density of 8.0g/cm³, a specific resistivity of 74µΩ•cm and a melting point of 1350°C.

### Embodiment 11

30 parts by weight of Fe metal blocks, 41 parts by weight of Cu metal blocks and 5 parts by weight of Sn metal blocks are molten at first, then 3 parts by weight of Al metal blocks are added and sequentially molten, uniform mixing is performed under high-speed electromagnet stirring, and the mixture is rapidly cast and then rapidly cooled to obtain an inert alloy anode 11. The inert alloy anode has a density of 8.1g/cm³, a specific resistivity of 68µΩ•cm and a melting point of 1370°C.

### Embodiment 12

23 parts by weight of Fe metal blocks, 60 parts by weight of Cu metal blocks, 14 parts by weight of Ni and 0.2 parts by weight of Sn metal blocks are molten at first, then 2.8 parts by weight of Al metal blocks are added and sequentially molten, and an inert alloy anode 12 is obtained by casting. The inert alloy anode has a density of 8.4g/cm³, a specific resistivity of 69µΩ•cm and a melting point of 1340°C.

### Embodiment 13

40 parts by weight of Fe metal blocks, 36 parts by weight of Cu metal blocks, 15 parts by weight of Ni and 5 parts by weight of Sn metal blocks are molten at first, then 4 parts by weight of Al metal blocks are added and sequentially molten, and an inert alloy anode 13 is obtained by casting. The inert alloy anode has a density of 8.15g/cm³, a specific resistivity of 69µΩ•cm and a melting point of 1369°C.

### Embodiment 14

36 parts by weight of Fe metal blocks, 47 parts by weight of Cu metal blocks, 14 parts by weight of Ni and 2.9 parts by weight of Sn metal blocks are molten at first, then 0.1 parts by weight of Al metal blocks are added and sequentially molten, and an inert alloy anode 14 is obtained by casting. The inert alloy anode has a density of 8.0g/cm³, a specific resistivity of 67.6µΩ•cm and a melting point of 1379°C.

### Embodiment 15

27 parts by weight of Fe metal blocks, 50 parts by weight of Cu metal blocks and 4 parts by weight of Sn metal blocks are molten at first, then 1 part by weight of Y metal blocks are added and sequentially molten, uniform mixing is performed under high-speed electromagnet stirring, and the mixture is rapidly cast and then rapidly cooled to obtain an inert alloy anode 15. The inert alloy anode has a density of 8.4g/cm³, a specific resistivity of 67µΩ•cm and a melting point of 1358°C.

### Embodiment 16

35 parts by weight of Fe metal blocks, 45 parts by weight of Cu metal blocks, 24 parts by weight of Ni and 4 parts by weight of Sn metal blocks are molten at first, then 2 parts by weight of Y metal blocks are added and sequentially molten, and an inert alloy anode 16 is obtained by casting. The inert alloy anode has a density of 8.1g/cm³, a specific resistivity of 70.9µΩ•cm and a melting point of 1375°C.

### Embodiment 17

25 parts by weight of Fe metal blocks, 50 parts by weight of Cu metal blocks and 4 parts by weight of Sn metal blocks are molten at first, then 3 parts by weight of Al metal blocks are added and sequentially molten, finally, 1 part by weight of Y metal blocks are added and molten, uniform mixing is performed under high-speed electromagnet stirring, and the mixture is rapidly cast and then rapidly cooled to obtain an inert alloy anode 17. The inert alloy anode has a density of 8.3g/cm³, a specific resistivity of 68.9µΩ•cm and a melting point of 1381°C.

### Embodiment 18

23 parts by weight of Fe metal blocks, 60 parts by weight of Cu metal blocks, 14 parts by weight of Ni and 0.9 parts by weight of Sn metal blocks are molten at first, then 0.1 parts by weight of Al metal blocks are added and sequentially molten, finally, 2 parts by weight of Y metal blocks are added and molten, mixing is performed, and the mixture is cast to obtain an inert alloy anode 18. The inert alloy anode has a density of 8.3g/cm³, a specific resistivity of 68µΩ•cm and a melting point of 1360°C.

### Embodiment 19

40 parts by weight of Fe metal blocks, 36 parts by weight of Cu metal blocks, 14.9 parts by weight of Ni and 5 parts by weight of Sn metal blocks are molten at first, then 4 parts by weight of Al metal blocks are added and sequentially molten, finally, 0.1 parts by weight of Y metal blocks are added and molten, mixing is performed, and the mixture is cast to obtain an inert alloy anode 19. The inert alloy anode has a density of 8.1g/cm³, a specific resistivity of 76.8µΩ•cm and a melting point of 1386°C.

### Embodiment 20

29 parts by weight of Fe metal blocks, 38.3 parts by weight of Cu metal blocks, 28 parts by weight of Ni and 0.2 parts by weight of Sn metal blocks are molten at first, then 3.5 parts by weight of Al metal blocks are added and sequentially molten, finally, 1 part by weight of Y metal blocks are added and molten, mixing is performed, and the mixture is cast to obtain an inert alloy anode 20. The inert alloy anode has a density of 8.2g/cm³, a specific resistivity of 70µΩ•cm and a melting point of 1365°C.

### Embodiment 21

40 parts by weight of Fe metal blocks, 36.5 parts by weight of Cu metal blocks, 18 parts by weight of Ni and 3 parts by weight of Sn metal blocks are molten at first, then 1.5 parts by weight of Al metal blocks are added and sequentially molten, finally, 1 part by weight of Y metal blocks are added and molten, mixing is performed, and the mixture is cast to obtain an inert alloy anode 21. The inert alloy anode has a density of 8.1g/cm³, a specific resistivity of 76.8µΩ•cm and a melting point of 1386°C.

### Embodiment 22

24.3 parts by weight of Fe metal blocks, 59 parts by weight of Cu metal blocks, 14 parts by weight of Ni and 0.2 parts by weight of Sn metal blocks are molten at first, then 2 parts by weight of Al metal blocks are added and sequentially molten, finally, 0.5 parts by weight of Y metal blocks are added and molten, mixing is performed, and the mixture is cast to obtain an inert alloy anode 22. The inert alloy anode has a density of 8.22g/cm³, a specific resistivity of 68.2µΩ•cm and a melting point of 1360°C.

In the aforementioned embodiment, 1 part by weight is 10g, and the inert anode alloy resulted from casting can be in any shape as required.

### Embodiment 23

40.01 parts by weight of Fe metal blocks, 35.9 parts by weight of Cu metal blocks and 0.19 parts by weight of Sn metal blocks are molten and then uniformly mixed under high-speed electromagnetic stirring, the mixture is rapidly cast and then rapidly cooled at a speed of 20-100°C/s to obtain an inert alloy anode 23 which is homogeneous in texture. The inert alloy anode has a density of 8.2g/cm³, a specific resistivity of 61µΩ•cm and a melting point of 1400°C.

### Embodiment 24

80 parts by weight of Fe metal blocks, 0.01 parts by weight of Cu metal blocks and 0.01 parts by weight of Sn metal blocks are molten and then uniformly mixed under high-speed electromagnetic stirring, the mixture is rapidly cast and then rapidly cooled at a speed of 20-100°C/s to obtain an inert alloy anode 24 which is homogeneous in texture. The inert alloy anode has a density of 7.5g/cm³, a specific resistivity of 82µΩ•cm and a melting point of 1369°C.

### Embodiment 25

60 parts by weight of Fe metal blocks, 25 parts by weight of Cu metal blocks and 0. 1 part by weight of Sn metal blocks are molten and then uniformly mixed under high-speed electromagnetic stirring, the mixture is rapidly cast and then rapidly cooled at a speed of 20-100°C/s to obtain an inert alloy anode 25 which is homogeneous in texture. The inert alloy anode has a density of 7.9g/cm³, a specific resistivity of 84µΩ•cm and a melting point of 1390°C.

### Embodiment 26

50 parts by weight of Fe metal blocks, 30 parts by weight of Cu metal blocks, 20 parts by weight of Mo and 0.05 parts by weight of Sn metal blocks are molten and then cast to obtain an inert alloy anode 26. The inert alloy anode has a density of 8.4g/cm³, a specific resistivity of 78µΩ•cm and a melting point of 1370°C.

### Embodiment 27

40.01 parts by weight of Fe metal blocks, 35.9 parts by weight of Cu metal blocks, 70 parts by weight of Ni and 0.01 parts by weight of Sn metal blocks are molten and then cast to obtain an inert alloy anode 27. The inert alloy anode has a density of 8.5g/cm³, a specific resistivity of 68µΩ•cm and a melting point of 1360°C.

### Embodiment 28

80 parts by weight of Fe metal blocks, 0.01 parts by weight of Cu metal blocks, 28.1 parts by weight of Ni and 0.19 parts by weight of Sn metal blocks are molten and then cast to obtain an inert alloy anode 28. The inert alloy anode has a density of 7.7g/cm³, a specific resistivity of 76.8µΩ•cm and a melting point of 1386°C.

### Embodiment 29

71.88 parts by weight of Fe metal blocks, 0.01 parts by weight of Cu metal blocks, 28.1 parts by weight of Ni and 0.01 parts by weight of Sn metal blocks are molten and then cast to obtain an inert alloy anode 29. The inert alloy anode has a density of 8.2g/cm³, a specific resistivity of 72µΩ•cm and a melting point of 1350°C.

### Embodiment 30

40.01 parts by weight of Fe metal blocks, 31.88 parts by weight of Cu metal blocks, 28.1 parts by weight of Ni and 0.01 parts by weight of Sn metal blocks are molten and then cast to obtain an inert alloy anode 30. The inert alloy anode has a density of 8.1g/cm³, a specific resistivity of 70µΩ•cm and a melting point of 1330°C.

### Embodiment 31

40 parts by weight of Fe metal blocks, 0.02 parts by weight of Cu metal blocks, 59.97 parts by weight of Ni and 0.01 parts by weight of Sn metal blocks are molten and then cast to obtain an inert alloy anode 31. The inert alloy anode has a density of 8.2g/cm³, a specific resistivity of 73µΩ•cm and a melting point of 1340°C.

### Embodiment 32

45 parts by weight of Fe metal blocks, 4.81 parts by weight of Cu metal blocks, 50 parts by weight of Ni and 0.19 parts by weight of Sn metal blocks are molten and then cast to obtain an inert alloy anode 32. The inert alloy anode has a density of 8.0g/cm³, a specific resistivity of 74µΩ•cm and a melting point of 1350°C.

### Embodiment 33

60 parts by weight of Fe metal blocks, 35.9 parts by weight of Cu metal blocks and 0.1 parts by weight of Sn metal blocks are molten at first, then 4 parts by weight of Al metal blocks are added and sequentially molten, uniformly mixing is performed under high-speed electromagnetic stirring, and the mixture is rapidly cast and then rapidly cooled to obtain an inert alloy anode 33. The inert alloy anode has a density of 8.1g/cm³, a specific resistivity of 68µΩ•cm and a melting point of 1370°C.

### Embodiment 34

40.01 parts by weight of Fe metal blocks, 27.7 parts by weight of Cu metal blocks, 28.1 parts by weight of Ni and 0.19 parts by weight of Sn metal blocks are molten at first, then 4 parts by weight of Al metal blocks are added and sequentially molten, and an inert alloy anode 34 is obtained by casting. The inert alloy anode has a density of 8.4g/cm³, a specific resistivity of 69µΩ•cm and a melting point of 1340°C.

### Embodiment 35

71.88 parts by weight of Fe metal blocks, 0.005 parts by weight of Cu metal blocks, 28.1 parts by weight of Ni and 0.01 parts by weight of Sn metal blocks are molten at first, then 0.005 parts by weight of Al metal blocks are added and sequentially molten, and an inert alloy anode 35 is obtained by casting. The inert alloy anode has a density of 8.15g/cm³, a specific resistivity of 69µΩ•cm and a melting point of 1369°C.

### Embodiment 36

40.01 parts by weight of Fe metal blocks, 31.88 parts by weight of Cu metal blocks, 25.01 parts by weight of Ni and 0.1 parts by weight of Sn metal blocks are molten at first, then 3 parts by weight of Al metal blocks are added and sequentially molten, and an inert alloy anode 36 is obtained by casting. The inert alloy anode has a density of 8.0g/cm³, a specific resistivity of 67.6µΩ•cm and a melting point of 1379°C.

### Embodiment 37

66 parts by weight of Fe metal blocks, 31.88 parts by weight of Cu metal blocks and 0.01 parts by weight of Sn metal blocks are molten at first, then 2 parts by weight of Y metal blocks are added and sequentially molten, uniformly mixing is performed under high-speed electromagnetic stirring, and the mixture is rapidly cast and then rapidly cooled to obtain an inert alloy anode 37. The inert alloy anode has a density of 8.4g/cm³, a specific resistivity of 67µΩ•cm and a melting point of 1358°C.

### Embodiment 38

40 parts by weight of Fe metal blocks, 0.01 parts by weight of Cu metal blocks, 59.97 parts by weight of Ni and 0.01 parts by weight of Sn metal blocks are molten at first, then 0.01 parts by weight of Y metal blocks are added and sequentially molten, and an inert alloy anode 38 is obtained by casting. The inert alloy anode has a density of 8.1g/cm³, a specific resistivity of 70.9µΩ•cm and a melting point of 1375°C.

### Embodiment 39

62 parts by weight of Fe metal blocks, 31.88 parts by weight of Cu metal blocks and 0.19 parts by weight of Sn metal blocks are molten at first, then, 4 parts by weight of Al metal blocks are added and sequentially molten, finally, 2 parts by weight of Y metal blocks are added and molten, uniform mixing is performed under high-speed electromagnet stirring, and the mixture is rapidly cast and then rapidly cooled to obtain an inert alloy anode 39. The inert alloy anode has a density of 8.3g/cm³, a specific resistivity of 68.9µΩ•cm and a melting point of 1381°C.

### Embodiment 40

40 parts by weight of Fe metal blocks, 25.7 parts by weight of Cu metal blocks, 28.1 parts by weight of Ni and 0.19 parts by weight of Sn metal blocks are molten at first, then 4 parts by weight of Al metal blocks are added and sequentially molten, finally, 2 parts by weight of Y metal blocks are added and molten, mixing is performed, and the mixture is cast to obtain an inert alloy anode 40. The inert alloy anode has a density of 8.3g/cm³, a specific resistivity of 68µΩ•cm and a melting point of 1360°C.

### Embodiment 41

71.88 parts by weight of Fe metal blocks, 0.005 parts by weight of Cu metal blocks, 28.1 parts by weight of Ni and 0.01 parts by weight of Sn metal blocks are molten at first, then, 0.002 parts by weight of Al metal blocks are added and sequentially molten, finally, 0.003 parts by weight of Y metal blocks are added and molten, mixing is performed, and the mixture is cast to obtain an inert alloy anode 41. The inert alloy anode has a density of 8.1g/cm³, a specific resistivity of 76.8µΩ•cm and a melting point of 1386°C.

### Embodiment 42

36.92 parts by weight of Fe metal blocks, 31.88 parts by weight of Cu metal blocks, 28.1 parts by weight of Ni and 0.1 parts by weight of Sn metal blocks are molten at first, then 1 part by weight of Al metal blocks are added and sequentially molten, finally, 2 parts by weight of Y metal blocks are added and molten, mixing is performed, and the mixture is cast to obtain an inert alloy anode 42. The inert alloy anode has a density of 8.2g/cm³, a specific resistivity of 70µΩ•cm and a melting point of 1365°C.

### Embodiment 43

39.81 parts by weight of Fe metal blocks, 0.01 parts by weight of Cu metal blocks, 59.97 parts by weight of Ni and 0.01 parts by weight of Sn metal blocks are molten at first, then 0.1 parts by weight of Al metal blocks are added and sequentially molten, finally, 0.1 parts by weight of Y metal blocks are added and molten, mixing is performed, and the mixture is cast to obtain an inert alloy anode 43. The inert alloy anode has a density of 8.1g/cm³, a specific resistivity of 76.8µΩ•cm and a melting point of 1386°C.

### Embodiment 44

45 parts by weight of Fe metal blocks, 24.4 parts by weight of Cu metal blocks, 29 parts by weight of Ni and 0.1 parts by weight of Sn metal blocks are molten at first, then 1 part by weight of Al metal blocks are added and sequentially molten, finally, 0.5 parts by weight of Y metal blocks are added and molten, mixing is performed, and the mixture is cast to obtain an inert alloy anode 44. The inert alloy anode has a density of 8.22g/cm³, a specific resistivity of 68.2µΩ•cm and a melting point of 1360°C.

In the aforementioned embodiments 23-44, 1 part by weight is 100g, and the inert anode alloy resulted from casting can be in any shape as required.

### Comparative Example

The alloy powders containing 37wt% of Co, 18wt% of Cu, 19wt% of Ni, 23wt% of Fe and 3wt% of Ag are subjected to powder metallurgic process to obtain an anode, and before use, an oxide film is formed on the surface of the metal anode by pre-oxidization at 1000°C to obtain an inert alloy anode A.

### Test Example

The inert alloy anodes 1-44 and A are each taken as an anode, graphite is taken as a cathode, the anode and the cathode are vertically inserted into an electrolytic cell provided with a corundum liner, and the distance between the anode and the cathode is 3cm. The anode has a current density of 1.0A/cm² at 760°C, and is electrolyzed for up to 40 hours in an electrolyte having the components including 32wt% of sodium fluoride, 57wt% of aluminum fluoride, 3wt% of lithium fluoride, 4wt% of potassium fluoride and 4wt% of alumina, and the test results are shown in the Table below:

| Inert Alloy Anode | Cell Voltage (V) | Direct Current Consumption for Per Ton of Aluminum (kw•h) | Purity of Product Aluminum (%) |
|---|---|---|---|
| 1 | 3.10 | 10040 | 99.80 |
| 2 | 3.14 | 10170 | 99.81 |
| 3 | 3.22 | 10429 | 99.85 |
| 4 | 3.16 | 10235 | 99.80 |
| 5 | 3.10 | 10040 | 99.85 |
| 6 | 3.39 | 10979 | 99.82 |
| 7 | 3.15 | 10202 | 99.85 |
| 8 | 3.27 | 10591 | 99.85 |
| 9 | 3.18 | 10299 | 99.83 |
| 10 | 3.36 | 10882 | 99.81 |
| 11 | 3.28 | 10623 | 99.80 |
| 12 | 3.40 | 11000 | 99.82 |
| 13 | 3.32 | 10753 | 99.84 |
| 14 | 3.25 | 10526 | 99.82 |
| 15 | 3.12 | 10105 | 99.80 |
| 16 | 3.27 | 10591 | 99.81 |
| 17 | 3.35 | 10850 | 99.83 |
| 18 | 3.38 | 10947 | 99.80 |
| 19 | 3.16 | 10234 | 99.82 |
| 20 | 3.32 | 10753 | 99.83 |
| 21 | 3.10 | 10040 | 99.81 |
| 22 | 3.12 | 10105 | 99.82 |
| 23 | 3.11 | 10040 | 99.80 |
| 24 | 3.13 | 10159 | 99.81 |
| 25 | 3.21 | 10429 | 99.85 |
| 26 | 3.15 | 10236 | 99.80 |
| 27 | 3.11 | 10041 | 99.90 |
| 28 | 3.38 | 10979 | 99.82 |
| 29 | 3.14 | 10202 | 99.85 |
| 30 | 3.26 | 10591 | 99.91 |
| 31 | 3.17 | 10299 | 99.83 |
| 32 | 3.35 | 10879 | 99.81 |
| 33 | 3.27 | 10623 | 99.80 |
| 34 | 3.39 | 11000 | 99.82 |
| 35 | 3.33 | 10753 | 99.84 |
| 36 | 3.25 | 10526 | 99.82 |
| 37 | 3.12 | 10105 | 99.80 |
| 38 | 3.27 | 10591 | 99.81 |
| 39 | 3.35 | 10850 | 99.83 |
| 40 | 3.38 | 10945 | 99.80 |
| 41 | 3.16 | 10234 | 99.82 |
| 42 | 3.32 | 10753 | 99.83 |
| 43 | 3.10 | 10040 | 99.81 |
| 44 | 3.12 | 10110 | 99.82 |
| A | 4.48 | 14510 | 98.35 |

It can be seen from the test results of the aforementioned embodiments and the comparative example that in the process of aluminum electrolysis, the inert alloy anode in the present invention has a cell voltage much lower than that of the alloy anode in the comparative example, consequently, using the inert alloy anode in the present invention can reduce the power consumption in an aluminum electrolysis process remarkably, which further reduces energy waste and lower cost. Meanwhile, the inert alloy anode in the present invention can be used for producing aluminum products which meet the high-purity standard, i.e. the purity of these aluminum products can be over 99.8, which meets the national primary aluminum standard.

## Claims

1. An inert alloy anode for aluminum electrolysis, comprising Fe, Cu, Ni and Sn, wherein the content of Fe is 23-40wt%, the content of Cu is 36-60wt%, the content of Ni is 14-28wt% and the content of Sn is 0.2-5wt%, or the content of Fe is 40.01-71.88wt%, the content of Cu is 0.01-31.88wt%, the content of Ni is 28.1-59.97wt% and the content of Sn is 0.01-0.19wt%.

2. The inert alloy anode according to claim 1, comprising Fe, Cu, Ni, Sn and Al, wherein the content of Fe is 23-40wt%, the content of Cu is 36-60wt%, the content of Ni is 14-28wt%, the content of Al is more than zero and less than or equal to 4wt% and the content of Sn is 0.2-5wt%, or the content of Fe is 40.01-71.88wt%, the content of Cu is 0.01-31.88wt%, the content of Ni is 28.1-59.97wt%, the content of Al is more than zero and less than or equal to 4wt% and the content of Sn is 0.01-0.19wt%.

3. The inert alloy anode according to claim 2,
being composed of Fe, Cu, Ni, Sn, Al and Y, wherein the content of Fe is 23-40wt%, the content of Cu is 36-60wt%, the content of Ni is 14-28wt%, the content of Al is more than zero and less than or equal to 4wt%, the content of Y is more than zero and less than or equal to 2wt% and the content of Sn is 0.2-5wt%, or the content of Fe is 40.01-71.88wt%, the content of Cu is 0.01-31.88wt%, the content of Ni is 28.1-59.97wt%, the content of Al is more than zero and less than or equal to 4wt%, the content of Y is more than zero and less than or equal to 2wt% and the content of Sn is 0.01-0.19wt%.

4. A preparing method of the inert alloy anode according to claim 1, comprising the following steps:
melting and mixing the metals Fe, Cu, Ni and Sn and then casting the mixture to obtain the inert alloy anode.

5. A preparing method of the inert alloy anode according to claim 2 or 3, comprising the following steps:
melting the metals Fe, Cu, Ni and Sn at a ratio according to claim 2 or 3 at first, then adding and melting the metal Al or Y at a ratio according to claim 2 or 3, and uniformly mixing,
or adding and melting the metal Al at a ratio according to claim 3 at first, then adding and melting the metal Y at a ratio according to claim 3, uniformly mixing, and casting the mixture to obtain the inert alloy anode.

## Patentansprüche

1. Inerte Legierungsanode für die Aluminiumelektrolyse,
umfassend Fe, Cu, Ni und Sn, wobei der Gehalt an Fe 23-40 Gew.-% beträgt, der Gehalt an Cu 36-60 Gew.-% beträgt, der Gehalt an Ni 14-28 Gew.-% beträgt und der Gehalt an Sn 0,2-5 Gew.-% beträgt oder der Gehalt an Fe 40,01-71,88 Gew.-% beträgt, der Gehalt an Cu 0,01-31,88 Gew.-% beträgt, der Gehalt an Ni 28,1-59,97 Gew.-% beträgt und der Gehalt an Sn 0,01-0,19 Gew.-% beträgt.

2. Inerte Legierungsanode nach Anspruch 1,
umfassend Fe, Cu, Ni, Sn und Al, wobei der Gehalt an Fe 23-40 Gew.-% beträgt, der Gehalt an Cu 36-60 Gew.-% beträgt, der Gehalt an Ni 14-28 Gew.-% beträgt, der Gehalt an Al größer als null und kleiner oder gleich 4 Gew.-% ist und der Gehalt an Sn 0,2-5 Gew.-% beträgt oder der Gehalt an Fe 40,01-71,88 Gew.-% beträgt, der Gehalt an Cu 0,01-31,88 Gew.-% beträgt, der Gehalt an Ni 28,1-59,97 Gew.-% beträgt, der Gehalt an Al größer als null und kleiner oder gleich 4 Gew.-% ist und der Gehalt an Sn 0,01-0,19 Gew.-% beträgt.

3. Inerte Legierungsanode nach Anspruch 2,
umfassend Fe, Cu, Ni, Sn, Al und Y, wobei der Gehalt an Fe 23-40 Gew.-% beträgt, der Gehalt an Cu 36-60 Gew.-% beträgt, der Gehalt an Ni 14-28 Gew.-% beträgt, der Gehalt an Al größer als null und kleiner oder gleich 4 Gew.-% ist, der Gehalt an Y größer als null und kleiner oder gleich 2 Gew.-% ist und der Gehalt an Sn 0,2-5 Gew.-% beträgt oder der Gehalt an Fe 40,01-71,88 Gew.-% beträgt, der Gehalt an Cu 0,01-31,88 Gew.-% beträgt, der Gehalt an Ni 28,1-59,97 Gew.-% beträgt, der Gehalt an Al größer als null und kleiner oder gleich 4 Gew.-% ist, der Gehalt an Y größer als null und kleiner oder gleich 2 Gew.-% ist und der Gehalt an Sn 0,01-0,19 Gew.-% beträgt.

4. Herstellungsverfahren für die inerte Legierungsanode nach Anspruch 1, das die folgenden Schritte umfasst:
Schmelzen und Mischen der Metalle Fe, Cu, Ni und Sn und dann Gießen der Mischung zum Erhalt der inerten Legierungsanode.

5. Herstellungsverfahren für die inerte Legierungsanode nach Anspruch 2 oder 3, das die folgenden Schritte umfasst:
zunächst Schmelzen der Metalle Fe, Cu, Ni und Sn in einem Verhältnis gemäß Anspruch 2 oder 3, dann Zugeben und Schmelzen des Metalls Al oder Y in einem Verhältnis gemäß Anspruch 2 oder 3 und einheitliches Mischen
oder zunächst Zugeben und Schmelzen des Metalls Al in einem Verhältnis gemäß Anspruch 3 und dann Zugeben des Metalls Y in einem Verhältnis gemäß Anspruch 3, einheitliches Mischen und Gießen der Mischung zum Erhalt der inerten Legierungsanode.

## Revendications

1. Anode en alliage inerte pour l'électrolyse d'aluminium,
comprenant du Fe, du Cu, du Ni et du Sn, dans laquelle la teneur du Fe est de 23-40 % en poids, la teneur du Cu est de 36-60 % en poids, la teneur du Ni est de 14-28 % en poids et la teneur du Sn est de 0,2-5 % en poids ou la teneur du Fe est de 40,01-71,88 % en poids, la teneur du Cu est de 0,01-31,88 % en poids, la teneur du Ni est de 28,1-59,97 % en poids et la teneur du Sn est de 0,01-0,19 % en poids.

2. Anode en alliage inerte selon la revendication 1, comprenant du Fe, du Cu, du Ni, du Sn et de l'Al, dans laquelle la teneur du Fe est de 23-40 % en poids, la teneur du Cu est de 36-60 % en poids, la teneur du Ni est de 14-28 % en poids, la teneur de l'Al est de plus de zéro à 4 % en poids ou moins et la teneur du Sn est de 0,2-5 % en poids ou la teneur du Fe est de 40,01-71,88 % en poids, la teneur du Cu est de 0,01-31,88 % en poids, la teneur du Ni est de 28,1-59,97 % en poids, la teneur de l'Al est de plus de zéro à 4 % en poids ou moins et la teneur du Sn est de 0,01-0,19 % en poids.

3. Anode en alliage inerte selon la revendication 2, qui est composée de Fe, de Cu, de Ni, de Sn, d'Al et de Y, dans laquelle la teneur du Fe est de 23-40 % en poids, la teneur du Cu est de 36-60 % en poids, la teneur du Ni est de 14-28 % en poids, la teneur de l'Al est de plus de zéro à 4 % en poids ou moins, la teneur de Y est de plus de zéro à 2 % en poids ou moins et la teneur du Sn est de 0,2-5 % en poids ou la teneur du Fe est de 40,01-71,88 % en poids, la teneur du Cu est de 0,01-31,88 % en poids, la teneur du Ni est de 28,1-59,97 % en poids, la teneur de l'Al est de plus de zéro à 4 % en poids ou moins, la teneur de Y est de plus de zéro à 2 % en poids ou moins et la teneur du Sn est de 0,01-0,19 % en poids.

4. Procédé de préparation de l'anode en alliage inerte selon la revendication 1, comprenant les étapes suivantes :
la fusion et le mélange des métaux Fe, Cu, Ni et Sn puis le coulage du mélange pour obtenir l'anode en alliage inerte.

5. Procédé de préparation de l'anode en alliage inerte selon la revendication 2 ou 3, comprenant les étapes suivantes :
d'abord la fusion des métaux Fe, Cu, Ni et Sn en une proportion selon la revendication 2 ou 3, puis l'ajout et la fusion du métal Al ou Y en une proportion selon la revendication 2 ou 3 et le mélange uniforme
ou d'abord l'ajout et la fusion du métal Al en une proportion selon la revendication 3, puis l'ajout et la fusion du métal Y en une proportion selon la revendication 3, le mélange uniforme et le coulage du mélange pour obtenir l'anode en alliage inerte.
